

# United States Patent [19]

von der Eltz et al.

[11] B 3,918,897

[45] Nov. 11, 1975

[54] **PROCESS FOR THE SINGLE-BATH DYEING OF UNMODIFIED POLYOLEFIN FIBERS WITH METAL-CONTAINING PHTHALOCYANINE**

[75] Inventors: **Hans-Ulrich von der Eltz**, Frankfurt am Main; **Armand Lehinant**, Offenbach am Main; **Hans-Peter Maier**, Sulzbach, Taunus, all of Germany

[73] Assignee: **Hoechst Aktiengesellschaft**, Frankfurt am Main, Germany

[22] Filed: Mar. 1, 1973

[21] Appl. No.: 336,902

[44] Published under the Trial Voluntary Protest Program on January 28, 1975 as document no. B 336,902.

[30] **Foreign Application Priority Data**

Mar. 7, 1972 Germany..... 2210879

[52] U.S. Cl..... 8/62; 8/1 XA; 8/30;

8/1; 8/169; 8/173; 8/180

[51] Int. Cl.<sup>2</sup> ..... D06P 1/14

[58] Field of Search ..... 8/1 XA, 180, 30, 1 S, 83, 8/62

[56]

## References Cited

### UNITED STATES PATENTS

3,097,044 7/1969 Skeuse ..... 8/30 X  
3,454,568 7/1969 Fuchs ..... 8/1 S

Primary Examiner—Donald Levy  
Attorney, Agent, or Firm—Curtis, Morris & Safford

[57]

## ABSTRACT

Process for the single-bath dyeing or printing of unmodified polyolefin fibers with metal-containing phthalocyanine dyestuffs, by reacting under high-temperature dyeing conditions on these textile materials aqueous liquors or printing pastes containing cationically modified phthalocyanine dyestuffs in the presence of a dispersion system on the basis of polyglycol ethers.

10 Claims, No Drawings

**PROCESS FOR THE SINGLE-BATH DYEING OF UNMODIFIED POLYOLEFIN FIBERS WITH METAL-CONTAINING PHTHALOCYANINE**

The present invention relates to a process for the single-bath dyeing of unmodified polyolefin fibers with metal-containing phthalocyanine dyestuffs.

It is known that unmodified polyolefin fibers, for example, polypropylene fibers, are, generally, difficult to dye by direct dyeing methods. Besides the immediate dyeing of the spinning mass in the melt with pigment dyestuffs, the dyeing of piece goods made of such fibers with aqueous suspensions of pigment dyestuffs and curable binding systems is described which form a correspondingly coloured film layer fast to washing on the fiber surface when being heated. Disperse dyes used for dyeing polyester fibers and other hydrophobic fibers, however, yield under comparable thermal conditions only very fair dyeings when being fixed the yield of which is unproportioned with respect to the amount of dyestuff used.

Various methods for the modification of the polyolefin material allow to improve the dye receptivity of the fiber considerably. For example, nitrogen-containing copolymers having a basic effect are introduced into the spinning melts of the fibrous ground substance of which the fibers consist and so anchored in the macromolecule. The fibers so modified then have affinity towards the anionic dyestuffs. Polypropylene can also be modified in such a manner that compounds of such metals which can form fast colour lakes with metallizable dyestuffs are incorporated into the mass or fiber. Thus, the fiber properties are influenced either by a metal-containing copolymer or by special after-treatment operations of the finished, unmodified fibrous material before dyeing, for example, as described in German Auslegeschriften Nos. 1,297 577, 1,469 600 and 1,619 601. But each of these processes for the modification of polyolefins requires additional operational expenditure which makes the fiber more expensive and sometimes inadvertently affects the physical properties of the fiber, for example, by reducing its stability and elasticity or by increasing its inflammability.

It was, now, found, that unmodified polyolefin fibers, preferably polypropylene fibers, can be dyed or printed in a single-bath operation with metal-containing phthalocyanine dyestuffs when allowing aqueous liquors or printing pastes containing cationically modified phthalocyanine dyestuffs to act under high temperature dyeing conditions, on the textile materials mentioned in the presence of a dispersion system on the basis of polyglycol ethers.

The present invention is based on the observation that the dyestuffs mentioned have a technically useful affinity towards the strongly hydrophobic, unmodified polyolefin fibers when they are present in a certain state of dispersion and are applied under adequate thermal conditions. Under these conditions, the dyeings or prints can be effected according to the process claimed using the exhaustion method, the pad-steaming method or a printing method together with steam fixation of the dyes. Taking into account a technical safety zone at a distance from the softening temperature of the fiber (150° - 155°C), the temperatures required are within the range of from 120° to 135°C, preferably about 130°C; the period of action is of 20 to 40 minutes, preferably of about 30 minutes, with the pad-

steaming and the print-steaming method, and of 50 to 70 minutes, preferably about 60 minutes, with the exhaustion method. It could not be expected that these conditions had been sufficient for the process of the invention to obtain a colour intensity which corresponded to the amount of dyestuff used.

The modified phthalocyanine dyestuffs to be used for carrying out the dyeings according to the new method contain as cationic radicals especially quaternary ammonium groups and are described in detail in literature. They are metal-containing phthalocyanine derivatives which contain 2 to 4 quaternary ammonium groups linked over methylene bridges to the benzene nuclei of the molecule. In these products the complex-bound metals to be considered are nickel, cobalt and, above all, copper. The quaternary nitrogen atom of the salt-forming radical carries identical or different, lower alkyl- or hydroxyalkyl groups; the anionic constituent is represented by the hydroxyl ion or the anion of an inorganic or organic acid, especially the acetate. Compounds of this type are described, for example, in German Pat. No. 1,220,065. Among the class of the phthalocyanine compounds which are water-soluble due to their salt-like substituents, the dyestuff of the formula



is particularly suitable.

To carry out the process of the invention, it is essential that the dyestuff is suitably distributed in the liquid which allows a diffusion into and thus an absorption by the fiber, at best by means of an auxiliary mixture. This dispersion system essentially consists of a non-ionic auxiliary on the basis of alkyl- or alkylaryl-polyglycol ethers or oxethylated fatty acid polyglycol esters, preferably a reaction product of 1 mol of isotridecyl alcohol with 8 mols of ethylene oxide, which is combined in the exhaustion method with anionic protective colloids having a dispersing effect, preferably those on the basis of lignin-sulfonic acid, and in the pad-steaming or print-steaming method with non-ionic protective colloids having a thickening effect, preferably a completely etherified locust bean flour.

When carrying out the process of the invention it was surprising that the simultaneous use of auxiliaries which split off acids under the action of heat (acid-yielding agent), for example, of the type of the monohalogenoacetates of alkali metals, preferably sodium monochloroacetate, or of the type of the chromium(III)-acetato-sulfate of the formula



promotes the fixation of the dyestuffs and thus the colour yield distinctly. Apparently, in the first phase of dyeing, the dyestuff is concentrated at the surface of the fiber towards which it has marked affinity already

at lower temperatures because of its cationic side chain. When the temperatures mentioned are reached, diffusion of the dyestuff from the surface to the interior of the fiber occurs. There is no doubt that the cationic group can be split off in this case. Such a reaction can be concluded from the efficiency of the acid-yielding agent (at least partially).

The following Examples illustrate the invention.

### EXAMPLE 1

Flock material of unmodified polypropylene fibers was dyed in a dyeing apparatus under high-temperature conditions, with a goods-to-liquor ratio of 1 : 20, for 60 minutes with an aqueous liquid which contained, calculated on the weight of the dry material,

2 % of a cationically modified phthalocyanine dyestuff of the formula



(CuPc = copper phthalocyanine)

4 % of an anionic protective colloid on the basis of lignin-sulfonic acid and

1 % of the reaction product of 1 mol of isotridecyl alcohol with 8 mols of ethylene oxide.

After dyeing, the material so obtained was subjected to rinsing and soaping in usual manner.

A brilliant fast turquoise dyeing was obtained.

### EXAMPLE 2

Piece-goods of unmodified polypropylene fibers were padded, with a liquor-pick-up of 70 % by weight, with a liquid at room temperature which contained per liter of water

20 g of the dyestuff mentioned in Example 1,

5 g of the reaction product of 1 mol of isotridecyl alcohol with 8 mols of ethylene oxide and

10 g of a 2 % aqueous solution of a completely etherified locust bean flour.

After the application of the dyestuff the material so treated was dried, steamed in a pressure steamer at 130°C for 30 minutes and then rinsed and finished in the usual manner.

A fast, brilliant turquoise dyeing was obtained.

When proceeding by this method prints can also be effected on the material.

### EXAMPLE 3

Dyeing was carried out in an analogous manner as described in Example 1, using, however, concomitantly

2 % of sodium monochloroacetate

as acid-yielding agent in the exhaustion bath. In this case, the yield of dyestuff is perceptibly better than that obtained by the prescription given in Example 1.

### EXAMPLE 4

Dyeing was carried out in an analogous manner as described in Example 2, using, however, concomitantly,

20 g/l of chromium-(III)-acetato-sulfate in the padding liquor.

In this case, the yield of dyestuff obtained is perceptibly higher than that obtained according to Example 2.

When proceeding by this method prints can also be effected on the material.

We claim:

1. An exhaust process for the single-bath dyeing or printing of unmodified polypropylene fibers, with metal-containing phthalocyanine dyestuffs, which comprises treating said fibers under high temperature dyeing conditions with aqueous dispersions containing

a. metal-containing phthalocyanine dyestuffs having 2 to 4 quaternary ammonium groups linked over methylene bridges to the benzene nuclei of the phthalocyanine molecule,

b. alkyl or alkylene-polyglycol ether or oxethylated fatty acid polyglycol ester, and

c. anionic protective colloids comprising lignin-sulfonic acid.

2. A process as claimed in claim 1, wherein the dyestuffs are applied to the fibers for 50-70 minutes at a temperature ranging from 120° to 135°C, preferably about 130°C.

3. A process as claimed in claim 1 wherein the said phthalocyanine dyestuffs have the following formula



4. A process as claimed in claim 1, wherein the said dispersion contains a non-ionic auxiliary comprising the reaction product of one mol of iso-tridecyl alcohol with 8 mols of ethylene oxide in combination with anionic protective colloids based on lignin-sulfonic acid.

5. A process as claimed in claim 1, wherein additional substances are employed for improving the color yield of the dyeing liquors, said substances splitting off acid under the influence of heat.

6. A process as recited in claim 5, wherein as the said acid-yielding substance, monohaloacetates of alkali metals, preferably sodium monochloro-acetate, or chromium-(III)-acetato-sulfates of the formula



are used.

7. A pad-steaming or print steaming process for the single-bath dyeing or printing of unmodified polypropylene fibers, with metal-containing phthalocyanine dyestuffs, which comprises treating said fibers under high temperature dyeing conditions after padding or printing with aqueous dispersions containing

- a. metal-containing phthalocyanine dyestuffs having 2 to 4 quaternary ammonium groups linked over methylene bridges to the benzene nuclei of the phthalocyanine molecule,
- b. alkyl or alkylene-polyglycol ether or oxethylated 5 fatty acid polyglycol ester; and
- c. non-ionic protective colloids having a thickening effect comprising etherified locust bean flour.

8. A process as recited in claim 7 wherein the dye-stuffs are padded or printed on the fibers and these 10 paddings or prints are then steamed, with or without intermediate drying, in a pressure steamer at 120° to 135°C for 20 to 40 minutes.

9. A process as claimed in claim 7, wherein the said 15 phthalocyanine dyestuffs have the following formula



10. A process as recited in claim 7, wherein said dispersion contains a non-ionic auxiliary based on the reaction product of one mol of iso-tridecyl alcohol with 8 mols of ethylene oxide in combination with non-ionic protective colloids having a thickening effect and comprising a completely etherified locust bean flour.

\* \* \* \* \*

20

25

30

35

40

45

50

55

60

65